

April 2, 1940.

E. G. SEARY

2,196,036

SUBTRACTIVE PROCESS FOR COLOR PHOTOGRAPHY

Filed March 31, 1938

2 Sheets-Sheet 1



Ag → develop in a  
bromideless developer

rinse and expose to white light

5 minutes in  
 $1\text{--}5\%$   $\text{NH}_3 + \text{K}_4\text{Fe}(\text{CN})_6$

10 minute wash

3 minutes in 2%  $\text{FeCl}_3 + \text{HCl}$

wash

5 minutes in 1%  $\text{NH}_3$   
rinse

5 minutes in  
5%  $\text{NH}_3 + \text{K}_4\text{Fe}(\text{CN})_6$

rinse

$\text{K}_4\text{Fe}(\text{CN})_6 + \text{HAc}$

10 minute wash

3 minutes in 2%  $\text{VCl}_3 + \text{HCl}$

wash

5%  $\text{NH}_3$

rinse

develop  $\text{AgI}$  in a color  
developer for magenta

rinse

$\text{K}_4\text{Fe}(\text{CN})_6 + \text{HAc}$

rinse

chromic acid

wash

$\text{V}_4[\text{Fe}(\text{CN})_6]_3 + \text{AgCl}$

$\text{V}(\text{OH})_3$

$\text{V}(\text{OH})_3$

$\text{Fe}(\text{OH})_3$

$\text{Ag} + \text{Magenta color}$

$\text{V}_4[\text{Fe}(\text{CN})_6]_3$

$\text{Fe}_4[\text{Fe}(\text{CN})_6]_3$

yellow

magenta

blue

Eugene G. Seary  
INVENTOR

BY *Seary and Jordan*

HIS ATTORNEYS

April 2, 1940.

E. G. SEARY

2,196,036

SUBTRACTIVE PROCESS FOR COLOR PHOTOGRAPHY

Filed March 31, 1938

2 Sheets-Sheet 2

Fig. 2



rinse and expose to white light



10 minute wash



wash

remove AgCl,  
precipitate  
Fe(OH)<sub>3</sub> & V(OH)<sub>3</sub>



develop AgI in a  
color developer for  
magenta image

rinse



rinse



wash Eugene G. Seary  
INVENTOR

BY *Kathy and Johnine*

HIS ATTORNEYS

## UNITED STATES PATENT OFFICE

2,196,036

SUBTRACTIVE PROCESS FOR COLOR  
PHOTOGRAPHY

Eugene G. Seary, Binghamton, N. Y., assignor,  
by mesne assignments, to General Aniline &  
Film Corporation, New York, N. Y., a cor-  
poration of Delaware

Application March 31, 1938, Serial No. 199,093

9 Claims. (Cl. 95—2)

The present invention relates to a process for forming prints and transparencies in color, to the light-sensitive material employed in said process, and to the products produced thereby.

5 The method at present widely used for producing multi-color part pictures involves the exposure of a multi-pack in an ordinary camera to simultaneously produce black and white color-separation latent images. The separation images 10 are then converted into proper dye images by a "controlled diffusion" development. In this controlled diffusion method, chemical agents are permitted to diffuse to a limited extent into the tri-pack to effect the changes desired. As is evident, 15 the thickness of the layers of the tri-pack is quite small and as a result this process, to give proper color rendition, requires the exercise of the greatest care and skill. In fact such skill is necessary that it is impossible for anyone other than the 20 laboratories actively engaged in the processing work to convert the latent images into multi-color pictures. It is also manifest that in view of the care required the cost of processing is relatively high. This method is, therefore, open to objection 25 for these reasons.

It is known that silver halides, i. e. the chloride, iodide and bromide, differ considerably as regards their solubility in ammoniacal solutions. Thus silver chloride is the most soluble of the three, 30 being about twenty times as soluble as silver bromide. Silver iodide, on the other hand, is the least soluble of the three, being only about one hundredth as soluble as silver bromide. By taking advantage of these differences in solubility of 35 these silver halides, I have devised a process for producing colored prints and transparencies which avoids the objections which manifest themselves in the process previously mentioned. My process involves the utilization of a multi-pack 40 in which the emulsions of at least two of the layers contain a different silver halide. Thus the light-sensitive material may be a tri-pack with a layer of silver chloride, a layer of silver bromide and a layer of silver iodide, a tri-pack with two 45 layers of silver bromide and one of silver iodide, a bi-pack with a layer of silver bromide and one of silver iodide, and the like. After exposure, the light-sensitive material is processed while using 50 soluble ferrocyanides with ammoniacal solutions of different concentrations and while effecting the desired changes by relying upon the differences in solubility between the silver halides of said emulsion layers.

It is an object of the present invention to produce pictures in color wherein a multi-pack, hav-

ing emulsion layers of different silver halides, is employed.

It is a further object of my invention to provide a process involving the use of soluble ferrocyanides in ammoniacal solutions of different 5 concentrations in treating an exposed light-sensitive material having layers containing different silver halides.

It is a further object of my invention to provide a process for forming multi-color part pictures in which it is unnecessary to carefully control the degree of diffusion of the processing 10 agents into the light-sensitive material.

A further object of my invention involves a light-sensitive material in the form of a multi- 15 pack in which at least two of the layers contain different silver halides.

Other important objects will be seen from the detailed description following hereafter.

As previously stated, my process relies for its 20 efficacy upon the utilization of a multi-pack which may have a base of paper, cellulose nitrate, cellulose acetate or the like, in which at least two layers carry a different silver halide gelatin emulsion. The particular manner of compounding the 25 light-sensitive material from the standpoint of arranging the layers on the base and of arranging the order of the different halide layers, may be varied to a considerable extent. For instance all three layers may be positioned on one side of the 30 base or two layers may be located on one side and one layer on the opposite side. When all three layers are on the same side of the base, three different silver halide layers are required. These may be arranged so that the layer adjacent 35 the base is silver chloride, the outermost layer is silver bromide and the intermediate layer silver iodide.

The yellow and blue color is imparted to the proper layers by means of inorganic pigments. 40 For this purpose I prefer the ferrocyanides which are formed in situ during the processing of the film. Thus ferric ferrocyanide may be used for producing the blue color and vanadium ferrocyanide for producing the yellow color. It is 45 also possible to produce the red color by means of a ferrocyanide pigment such as uranium ferrocyanide. Similarly nickel di-methyl glyoxime may be used for this purpose. However, due to the lack of brilliance of the red pigments, it is 50 advisable for best results to produce the red color by the process known as "color development". A discussion of color development may be found on pages 404-407 of "History of Three-Color Photography" by Wall. On page 406, compounds 55

suitable for producing color in this way are mentioned. Examples of compounds which may be employed for producing the red color are methyl phenyl pyrazolone, methyl diphenyl pyrazolone, 5 benzyl cyanide and the like. The color components may be incorporated either in the emulsion or added to the developer, the latter procedure being preferred. The developers are those of the paraphenylenediamine type such as para- 10 phenylene diamine, dimethyl paraphenylenediamine, ethyl paraphenylenediamine, diethyl paraphenylenediamine and the like.

As is usual in color photography, my multi-packs, especially in those layers designed to register 15 the red and green color sensations of the object, are sensitized to effect color separation in said layers. Dyestuffs suitable for this purpose are well known in the art, a list of such dyes being given, for instance, on pages 252-263 of "History 20 of Three-Color Photography" by Wall. I prefer, in forming my multi-packs, to sensitize for the red region with Pinacyanol and for the green region with Eosin.

The facility with which my process may be 25 accomplished may be perceived by considering its application in its general aspects to, for example, a light-sensitive material having a gelatino-silver chloride layer, sensitized to red, positioned on a base, a gelatino silver iodide emulsion layer sensitized to green positioned on said first layer, and a gelatino-silver bromide emulsion layer not specially sensitized, positioned on said second layer. Said light-sensitive material is exposed 30 and developed in the ordinary way after which it is subjected to the action of white light. The developer employed may be any developer. Should silver chloride be present in one of the emulsion layers, the developer should in addition be free from bromide. The light-sensitive material is now subjected to the action of a weak ammoniacal solution containing a soluble ferrocyanide, i. e. an alkali-metal ferrocyanide, the strength of said solution being such that, while it will dissolve silver chloride, it has no effect upon 45 silver iodide or bromide. Silver ferrocyanide is produced in the silver chloride layer by this treatment as a result of the dissolution of the silver chloride by the ammonia and its reaction with said ferrocyanide. The silver ferrocyanide is then converted to ferric ferrocyanide by an acid treatment with ferric chloride. The silver bromide layer is now colored by means of vanadium ferrocyanide by dissolving the silver bromide with a stronger ammoniacal solution than that used in 50 the first treatment, said solution also containing an alkali metal ferrocyanide, the silver ferrocyanide thus obtained being converted to vanadium ferrocyanide by an acid treatment with vanadium chloride. A silver and dye image is next 55 formed in the silver iodide layer by development in a paraphenylenediamine developer containing a color component which is capable of reacting with the oxidation product of the developer to produce a dye imparting a reddish color. By dissolving the silver from the light-sensitive material 60 by means of a bleach such as chromic acid, there is obtained a transparency in which the outer layer is colored yellow, the inner layer is colored blue and the intermediate layer magenta.

70 My invention will be illustrated in greater detail by means of the following examples and the accompanying self-explanatory drawings, in which

Fig. 1 discloses the steps of processing a tri-pack having a paper base, and

Fig. 2 the processing of a film.

Example 1.—The tri-pack of Fig. 1 comprises a paper support 1 upon which is superimposed a red sensitized silver chloride gelatin emulsion 2, a green sensitive silver iodide gelatin emulsion 3 and 5 a non-sensitized silver bromide gelatin emulsion 4. The latter emulsion contains an agent for imparting a yellow color to the emulsion for the purpose of preventing blue light from passing to the green and red sensitive emulsion layers. If 10 desired, the same result may be obtained by interposing a yellow dye layer between layers 3 and 4. For this purpose tartrazine which is discharged during development has been employed although it is to be borne in mind that other dyestuffs usually employed in the art for this purpose may be utilized. The paper is exposed either directly or through filters to the action of light, whereupon there is produced in the lowermost layer a latent image of the red sensations of the object, 15 in the intermediate layer a latent image of the green sensations of the object and in the outermost layer a latent image of the blue sensations of the object. The paper is next developed in a bromideless developer such as amidol, rinsed, 20 and subjected to the action of white light. After the exposure the silver chloride emulsion layer is treated for about 5 minutes in a .1 to .5% solution of ammonia containing added potassium ferrocyanide. Dissolution of the silver chloride 25 takes place with the immediate precipitation of silver ferrocyanide through reaction of the dissolved chloride with the added potassium ferrocyanide. A washing in water is interpolated between this step and the succeeding step wherein the paper is subjected for a short time, say, about 3 minutes, to the action of a solution containing about 2% of ferric chloride acidified with hydrochloric acid. A reaction ensues between the silver ferrocyanide and the iron chloride resulting 30 in the formation of ferric ferrocyanide, silver chloride being regenerated. The silver chloride is removed by a treatment in a dilute ammoniacal solution, a treatment for about 5 minutes in a 1% ammonia solution being efficacious in accomplishing 35 this result. As a result of the action of the ammonia, the ferric ferrocyanide is converted to ferric hydroxide. By-products of the reaction are removed by a rinse after which the silver bromide emulsion layer is acted upon for a short 40 time, say about 5 minutes with a stronger ammoniacal solution than that previously used. Preferably a 5% solution is employed at this stage. The ammoniacal solution contains potassium ferrocyanide which reacts with the silver 45 bromide to produce silver ferrocyanide. Following a rinsing step, the ferric hydroxide in the lowermost layer 2 is reconverted to ferric ferrocyanide by means of an acid potassium ferrocyanide bath. After washing for a short time, the 50 paper is next treated for about three minutes in a 2% vanadium chloride solution containing free hydrochloric acid. Vanadium ferrocyanide, a light yellow compound, is thus produced in the outermost layer. The silver chloride produced 55 as a by-product in this reaction is removed by a treatment with 5% ammonia solution, whereby the ferrocyanides of iron and vanadium are converted to their respective hydroxides. After rinsing, the paper is then subjected to the action of 60 a p-phenylenediamine developer containing methyl phenyl pyrazolone. The products of oxidation produced by the reduction of the silver iodide in the intermediate layer thereupon react with the methyl phenyl pyrazolone to produce a 65 70 75

silver and dye image in this layer. The paper is next treated with acid potassium ferrocyanide to regenerate the vanadium and ferric ferrocyanides in layers 2 and 4. The silver is finally removed by 5 means of a chromic acid treatment whereby there is produced a transparency having superimposed layers colored blue, magenta and yellow respectively.

*Example 2.*—The film of Fig. 2 of the drawings, as there depicted, involves a departure from the paper of Fig. 1 in the arrangement and nature of the emulsion layers. In this modification the film base 1 has arranged on the entrant side of the film a silver bromide emulsion layer 2 containing a yellow dyestuff such as tartrazine. On the opposite side of said film base there are located two emulsion layers 3 and 4, layer 3 being a silver iodide emulsion sensitized for green, and layer 4 being a silver bromide emulsion sensitized for red. The light-sensitive material, after exposure, if desired behind filters, is developed in an amidol developer to produce white and black color-separation images. The film, after exposure to white light, is treated with a 25 5% ammoniacal solution containing about 5% potassium ferrocyanide, as a result of which the silver bromide in layers 2 and 4 is converted to silver ferrocyanide. After washing, layer 4 alone is subjected to the action of a 2% ferric chloride solution acidified with hydrochloric acid. In this way the silver ferrocyanide in layer 4 is converted into ferric ferrocyanide. The next step involves the treatment of layer 1 with a 2% vanadium chloride solution, acidified with hydrochloric acid to convert the silver ferrocyanide of this layer into vanadium ferrocyanide. The silver chloride which is produced in forming the ferric and vanadium ferrocyanides respectively, is removed with a, say about 5% ammonia solution subsequent to a washing of the film. In this removal of the silver chloride, the ferrocyanides of iron and vanadium are converted to ferric hydroxide and vanadium hydroxide respectively. The silver iodide layer 3 is now developed with a paraphenylenediamine developer containing methyl phenyl pyrazolone whereby the oxidation products of the diamine combine with the methyl phenyl pyrazolone to produce in this layer a silver and dye image. The film, following a rinsing operation, is subjected to the action of an acidified potassium ferrocyanide solution to cause regeneration of vanadium and ferric ferrocyanides from their respective hydroxides. By now bleaching out the silver with 55 chromic acid, a transparency having yellow, magenta and blue dye images is obtained. The same or similar procedure may be adopted in processing a film having 2 silver chloride- and one silver iodide- or one silver bromide-emulsions.

In referring to the solutions by which the silver salts are dissolved, I have typified the same as ammoniacal solutions. This term is to be construed as covering not only solutions of ammonia but in addition solutions of ammonium salts as well as solutions of amines. Examples of the ammonium salts are ammonium sulfate, ammonium acetate, ammonium chloride and the like. Examples of the amines are the alkylol amines such as ethanol amine, di-ethanol amine, tri-ethanol amine, propanol amine and the like, alkyl amines such as methyl amine, ethyl amine, propyl amine and the like, hydroxyl amines, etc. It is to be pointed out that for the purposes of 70 my invention the ammonium salts and the

amines function to produce the result desired although I prefer solutions of ammonia.

In the preceding examples, in lieu of removing the silver chloride by means of ammonium hydroxide at the times indicated, I also contemplate converting the ferric and vanadium ferrocyanides to their respective hydroxides by means of a dilute alkali such as sodium hydroxide, potassium hydroxide and the like, after which the silver chloride may be removed by dilute ammonia such as that having a concentration of about 1%. It should be understood that this and other modifications apparent to a person skilled in the art are within the scope of my invention. Thus instead of using separate layers 15 of different silver halide emulsions, I may employ a single layer in which the different silver halide emulsions are present in admixture with each other.

What I claim is:

1. In the process of producing multi-color pictures in which latent images are formed in a multi-layer gelatino-silver halide light-sensitive material in which the emulsion of one layer of said material is formed with a silver halide different from the silver halide used to form the emulsion of another layer of said material and in which the latent images are then developed in a black and white developer but not fixed, the improvement which comprises re-exposing the light-sensitive material to white light and subjecting the exposed light-sensitive material to the action of a soluble ferrocyanide in an ammoniacal solution of such strength that only one of the silver halides is dissolved and converted into silver ferrocyanide by the soluble ferrocyanide present.

2. In the process of producing multi-color pictures in which latent images are formed in a gelatino-silver halide light-sensitive material having three layers, the emulsion of one of said layers being formed with a silver halide different from the silver halide used to form the emulsion of at least one other layer and in which the latent images are then developed in a black and white developer but not fixed, the improvement which comprises re-exposing the light-sensitive material to white light, subjecting the light-sensitive material to the action of a soluble ferrocyanide in an ammoniacal solution of such strength that only one of said silver halides is dissolved and converted into silver ferrocyanide by the ferrocyanide present, and subjecting the light-sensitive material to the action of a soluble ferrocyanide in an ammoniacal solution of such strength that only one of said silver halides is dissolved and converted into silver ferrocyanide by the ferrocyanide present.

3. In the process of producing multi-color pictures in which latent images are formed in a gelatino-silver halide light-sensitive material having three layers, the emulsion of one of said layers being formed with a silver halide different from the silver halide used to form the emulsion of at least one other layer and in which the latent images are then developed in a black and white developer but not fixed, the improvement which comprises re-exposing the light-sensitive material to white light, subjecting the light-sensitive material to the action of a soluble ferrocyanide in an ammoniacal solution of such strength that only one of said silver halides is dissolved and converted into silver ferrocyanide by the ferrocyanide present, converting the silver ferrocyanide into ferric ferrocyanide and then

subjecting the light-sensitive material to the action of a soluble ferrocyanide in an ammoniacal solution of such strength that only one other of said silver halides is dissolved and converted into silver ferrocyanide by the ferrocyanide present.

5. The process of producing multi-color pictures which comprises exposing a multi-layer gelatino-silver halide light-sensitive material, in which the emulsion of one layer being formed 10 with a silver halide different from the silver halide used to form the emulsion of another layer, developing the latent images in a black and white developer and without fixing, exposing the light-sensitive material to white light, converting 15 the silver halide most soluble in ammonia into silver ferrocyanide by the action of a soluble ferrocyanide in an ammoniacal solution and converting the silver ferrocyanide into a colored ferrocyanide.
- 20 6. The process as defined in claim 4, wherein the multi-pack contains at least one silver bromide emulsion layer and a silver iodide emulsion layer.

- 25 7. The improvement defined in claim 2, wherein in the silver ferrocyanides in the separate layers are converted into ferric ferrocyanide and vanadium ferrocyanide and wherein a silver and dyestuff picture is produced in the third layer by color development.

7. The process of producing multi-color pictures by exposing a tripack in which at least one of the layers is a silver bromide emulsion and another of the layers is a silver iodide emulsion, developing the latent images in a black and white developer and without fixing, converting the silver bromide into silver ferrocyanide by an ammoniacal solution containing potassium ferrocyanide to which the silver iodide is inert, treating the light-sensitive material with a chloride selected from the class consisting of iron and vanadium to convert the silver ferrocyanide into a ferrocyanide selected from the class consisting of iron and vanadium, removing silver chloride by means of an ammoniacal solution having 15 no dissolving power on silver iodide, producing a silver and dyestuff image in the silver iodide layer by color development, reconverting the metal hydroxide formed in the silver chloride removal step to the corresponding ferrocyanide 20 by acidified potassium ferrocyanide and removing metallic silver.

8. The process as defined in claim 1, in which the ammoniacal solution is a solution of an ammonium salt.

25 9. The process as defined in claim 1, wherein the ammoniacal solution is a solution of an amine.

EUGENE G. SEARY.